# EUROPEAN PATENT SPECIFICATION

(11) **EP 4 508 270 B1**
(45) Date of publication and mention of the grant of the patent: **15.04.2026**
(21) Application number: 23716337.3
(22) Date of filing: 14.04.2023
(51) Int. Cl.: D21H 11/04, B32B 29/00, D21F 3/02, D21H 11/08, D21H 11/10, D21H 11/14, D21H 27/10, D21H 27/38

(54) **PRODUCTION OF PAPER- OR LINERBOARD**
HERSTELLUNG VON PAPIER- ODER DECKENPAPIER
PRODUCTION DE PAPIER OU DE CARTON DOUBLURE

(30) Priority: 14.04.2022 EP 22168616
(43) Date of publication of application: 19.02.2025
(73) Proprietor: Billerud Aktiebolag (publ), 169 27 Solna (SE)
(72) Inventor: NORDSTRÖM, Fredrik, 652 26 Karlstad (SE)
(74) Representative: Kransell & Wennborg KB
(86) International application number: PCT/EP2023/059830
(87) International publication number: WO 2023/198916

(56) References cited:
- EP-A1- 3 739 115
- WO-A1-2021/124040
- CN-A- 106 948 208
- CN-A- 110 904 734
- DE-A1- 102019 116 602
- US-A1- 2008 053 634
- US-A1- 2021 221 114

## Description

### TECHNICAL FIELD

The present disclosure relates to the field of production of paper- and linerboard.

### BACKGROUND

A machine for producing multi-layered paper- or linerboard has different sections. In the wet end of the paper machine, furnishes are prepared from pulps and additives (added to improve properties such as retention, dewatering and strength). In the forming/wire section, a multi-layered web is then formed from the furnishes. The multi-layered web is dewatered in the press section and dried in the drying section. Downstream the drying section, the multilayered web may be coated and/or calendered. When the multilayered web is both coated and calendered, calendering can be carried out upstream or downstream the coating step(s) or even between coating steps.

The pulps that can be used in the paperboard machine include virgin pulps, recycled pulps (i.e. pulps prepared from recycled paper and/or paperboard) and broke pulps (pulps of fibres recycled from downstream portions of the same process). Further, virgin pulps are typically divided into chemical pulps and mechanical pulps. Sulfate (kraft) pulp and sulfite pulp are examples of chemical pulp. Groundwood pulp, thermomechanical pulp (TMP) and chemi-thermomechanical pulp (CTMP) are examples of mechanical pulp. All these pulps can be made from hardwood, softwood or mixtures thereof. Further, the pulps can be bleached or unbleached.

A furnish for a particular layer typically comprise a mixture of different pulps. The properties of the final board product are not only a result of the pulp mixture of each furnish; they also depend on the degree of refining of the pulps, the types and amounts of additives and other operating conditions. However, the process for making paperboard cannot be designed with only the final properties in mind; runnability in the paper machine and energy consumption must also be taken into consideration.

WO2021124040 discloses a method to produce a linerboard exhibiting a high bending resistance and a high compression strength, which in turn provides high resistance to interflute buckling and sagging in a thereof formed corrugated board. This is achieved by the combination of an optimized fiber refining level of the furnish in each layer of the linerboard, the separate formation of the top layer and the use of a multi-layer headbox to form the two-layered ply. In addition, the linerboard made according to the provides good printing properties in a thereof produced corrugated board, especially in flexographic printing, without the fluting structure being negatively affected.

DE102019116602 discloses a machine for producing a fibrous material web, in particular a packaging paper or cardboard web. The machine comprises at least one, preferably two, double-felted shoe presses mounted one behind the other in the direction of movement of the web, and at least one single-felted shoe press mounted downstream of the two double-felted shoe presses in the direction of movement, particularly in the form of a smoothing press.

US2021221114 discloses a ply of a linerboard for corrugated board, which ply exhibits high strength properties and which enables the production of lightweight linerboards. The ply comprises 20-80 wt % CTMP from wood fibers and 80-20 wt % chemical pulp, calculated on the total fiber weight of said ply and strength additives chosen from the group of microfibrillated cellulose (MFC), anionic or cationic polymers and starch or combinations thereof. The ply exhibits a geometric SCT index of above 22 Nm/g and a density of below 680 kg/m3, preferably of below 650 kg/m3.

CN110904734 discloses a preparation method of a dark-streak anti-counterfeiting paperboard. The preparation method comprises the following steps: primarily dehydrating pulp through a forming plate, then performing dehydrating through a forming net under vacuum, and carrying out squeezing and drying to obtain the dark-streak anti-counterfeiting paperboard, wherein a bottom-layer pulp net speed difference is in a range of -5 to -20 m/min during dehydration treatment of the forming net, and the forming net is provided with a dark streak structure. It is stated that the method, compared to the prior art, has the following advantages: in the dehydration forming process, the forming net provided with dark streaks is adopted for dehydration treatment, so fibers are regularly distributed according to the darkstreaks, and therefore, the surface of a paper web has a partly-hidden and partly-visible dark streak effect; an anti-counterfeiting mark is high in concealment and distinguishability, and additional equipment is not needed for identification; the preparation method only needs to adopt conventional processes and equipment, so production cost is not increased, paper is not damaged at all, and continuous use is not affected; and the dark-streak anti-counterfeiting paperboard has the same advantages of high strength, easy degradability, repeated usability and the like as common paper.

US20080053634 discloses a method and a machine for producing a fiber web having a mass per unit area of less than 125 g/m2. The method includes applying a fluid application medium to the fibrous web. The fluid application medium being a liquid having a solids concentration of 15% or more. The machine for producing a fiber web includes a press section having at least one press nip and at least one application device structured and arranged to apply a liquid medium to one side of the fiber web at least one of immediately before the at least one press nip and in the at least one press nip.

### SUMMARY

The present disclosure aims to provide an efficient method of producing a paper- or linerboard of satisfactory properties.

Accordingly, the present disclosure provides a method of producing a paper- or linerboard having a grammage measured according to ISO 536:2019 of 170-310 g/m² and comprising a print layer, a middle layer and a back layer, wherein the middle layer is formed from a middle layer furnish comprising at least 30% by dry weight CTMP and at least 20% by dry weight broke pulp and the back layer is formed from a back layer furnish comprising at least 60% by dry weight of an unbleached kraft pulp, said method comprising the step of subjecting a multi-layered web at a speed of at least 600 m/min to pressing in a press section comprising a first and a second double-felted shoe press nip arranged in series, wherein the total press impulse of the double-felted shoe press nips is at least 95 kPa*s, preferably at least 100 kPa*s,
and wherein CTMP and broke pulp together constitute at least 65% by dry weight of the middle layer furnish
and wherein the press section comprises a further nip arranged downstream the double-felted shoe press nips, which further nip is a hard nip or a single-felted shoe press nip, in which single-felted shoe press nip the felt is contacting the back side and wherein the print layer is coated with a composition comprising at least one pigment and at least one binder, which coating step comprises a plurality of substeps, each applying a sublayer and wherein the total amount (dry weight) of coating applied in the coating step is 11-30 g/m²
and wherein the paper- or linerboard is subjected to hard nip calendering prior to the coating step but after a drying section
and wherein the method comprises no calendering step after the coating step
and wherein the pigment-coated the print side of the paper- or linerboard has a PPS 1.0 roughness measured according to ISO 8791-4:2013 (soft backing & 1000 kPa clamping pressure) of below 1.8 µm.

Compared to the prior art, this press impulse is high, which increases the press dryness (i.e. the dryness of the multilayered web exiting the press section). As a result, less steam is consumed in the drying section. The skilled person making paperboard is often reluctant to use high press impulses as they can densify the web to such an extent that inferior bending stiffness is obtained. However, the selection of an unbleached pulp for the back layer furnish and the inclusion of CTMP in the middle layer furnish make the web of the method of the present disclosure relatively insensitive to high press impulses. The press dryness is further increased by both shoe press nips being double-felted.

It is also shown herein that a method according to the present disclosure can improve printing surface properties.

### DETAILED DESCRIPTION

The present disclosure provides a method of producing a paper- or linerboard having a grammage measured according to ISO 536:2019 of 170-310 g/m².

The paper- or linerboard comprises a print layer, a middle layer and a back layer. In one embodiment, the paper- or linerboard comprises more than one middle layer.

The middle layer is formed from a middle layer furnish comprising at least 30% by dry weight CTMP. In case of more than one middle layer, each middle layer furnish preferably comprise at least 25% by dry weight CTMP. The CTMP of the middle layer(s) preferably has a Canadian Standard Freeness (CSF) measured according to ISO 5267-2:2001 of 525-625 ml, such as 550-600 ml. To reach such a CSF, the CTMP may be subjected to refining. If the CSF is too low, dewatering is impaired and density increases. If the CSF is too high, strength properties may be insufficient.

In one embodiment, the middle layer furnish comprises at least 40% by dry weight CTMP.

In addition to CTMP, the middle layer furnish comprises at least 20% by dry weight broke pulp, such as at least 30% by dry weight broke pulp. The broke pulp of the middle layer furnish preferably has a Schopper-Riegler number (°SR) of less than 35 (such as 26-34), more preferably less than 33 (such as 27-32). To reach such a °SR, the broke pulp may be subjected to refining. In the present disclosure, °SR is measured according to ISO 5267-1:1999.

In one embodiment, the CTMP and the broke pulp together constitute at least 65% by dry weight of the middle layer furnish, such as at least 75% by dry weight of the middle furnish.

The middle layer furnish may further comprises kraft pulp, such as softwood kraft pulp. This kraft pulp may have a relatively low °SR, such as 18-25, preferably 18-23.

The head box consistency of the middle layer furnish may be 0.15% - 0.42%, such as 0.25% - 0.40%.

The back layer is formed from a back layer furnish comprising an unbleached kraft pulp. The unbleached pulp of the back layer preferably has a °SR of 19-26, such as 20-25. To reach such a °SR, the unbleached pulp may be subjected to refining. If the °SR is too high, dewatering is impaired. If the °SR is too low, strength properties may be insufficient.

The unbleached pulp of the back layer is typically a softwood pulp.

The back layer furnish comprises at least 60% by dry weight of the unbleached pulp.

In addition to the unbleached pulp, the back layer furnish may comprise broke pulp. The broke pulp of the back layer furnish preferably has a °SR of less than 35 (such as 26-34), more preferably less than 33 (such as 27-32). To reach such a °SR, the broke pulp may be subjected to refining.

In one embodiment, the unbleached pulp and broke pulp together constitute at least 80 % by dry weight of the back layer furnish, such as at least 90 % by dry weight of the back layer furnish.

The head box consistency of the back layer furnish may be 0.12% - 0.25%.

The print layer furnish preferably comprises a mixture of hardwood kraft pulp and softwood kraft pulp, such as a mixture of bleached hardwood kraft pulp and bleached softwood kraft pulp. However, the print layer may also be unbleached.

Each of the kraft pulps of print layer furnish preferably has a °SR of 21-29. To reach such a °SR, the kraft pulps are typically subjected to refining.

In one embodiment, hardwood kraft pulp and softwood kraft pulp together constitute at least 80% by dry weight of the print layer furnish, such as at least 90% by dry weight of the print layer furnish.

The head box consistency of the print layer furnish may be 0.12% - 0.25%.

As understood by the skilled person, the above-mentioned furnishes form a multi-layered web in a forming section. A top former may be arranged to aid the dewatering of the middle layer in the forming section. Further, the formation of the middle layer preferably comprises the use of a breast roll shaker.

The method of the present disclosure comprises the step of subjecting the multi-layered web to pressing in a press section at a speed of at least 600 m/min, such as at least 650 m/min, such as at least 700 m/min, such as at least 750 m/min.

The press section comprises a first and a second double-felted shoe press nip arranged in series. As understood by the skilled person, the second double-felted shoe press nip is arranged downstream the first double-felted shoe press nip. Preferably the line load of the second double-felted shoe press nip is higher than the line load of the first double-felted shoe press nip.

The total press impulse of the double-felted shoe press nips is at least 95 kPa*s, preferably at least 100 kPa*s. An upper limit may be 150 kPa*s or 200 kPa*s
If the grammage is relatively high, such as 250-310 g/m², the speed of the multi-layered web is typically lower, which means that the press impulse can be higher, e.g. at least 105 kPa*s, such as at least 110 kPa*s.

The press section comprises a further nip arranged downstream the double-felted shoe press nips. The further nip is a non-felted hard nip or a single-felted shoe press nip. When the further nip is a non-felted hard nip, its line load may be in the range of 25-100 kN/m, such as 30-75 kN/m, such as 30-60 kN/m. The main purpose of such a hard nip is to smoothen the print side, which was in contact with a felt in the first and the second double-felted shoe press nip. When the further nip is a single-felted shoe press nip, the felt is contacting the back side. Thereby, the single-felted shoe press nip not only further dewaters the web, it also smoothens the print side, which - as mentioned above - was in contact with a felt in the first and the second double-felted shoe press nip.

The print layer of the paper- or linerboard is coated with a composition comprising at least one pigment and at least one binder. Accordingly, the method of the present disclosure further comprises a coating step. The coating step comprises a plurality of substeps, each applying a sublayer. The total amount (dry weight) of coating applied in the coating step is 11-30 g/m².

When pigment-coated, the print side of the paper- or linerboard of the present disclosure has a PPS 1.0 roughness of below 1.8 µm. A lower limit for this PPS 1.0 roughness may be 0.8 µm. In the present disclosure, PPS 1.0 roughness is measured according to ISO 8791-4:2013 (soft backing & 1000 kPa clamping pressure).

Prior to the coating step (but after the drying section), the paper- or linerboard is subjected to calendering to improve the coatability. Such calendering is hard nip calendering, which may be carried out at an elevated temperature. As an example, the surface temperature of a heated roll of the hard nip calender may be in the range of 100-250 °C.

The method of the present disclosure comprises no calendering step after the coating step, which typically saves bulk.

The density of the paper- or linerboard of the present disclosure may be below 810 kg/m³. If not coated with a pigment coating, the density may be below 800 kg/m³. In the present disclosure, density is measured according to ISO 534:2011.

### EXAMPLE 1

### Production of a ~200 g/m² WTL

A three-layer white-top linerboard (WTL) was produced in a full-scale paperboard machine. The layer design of the WTL was as follows: a print layer (58 g/m²), a back layer (45 g/m²), a middle layer (77 g/m²) and a pigment coating (20 g/m², applied onto the print layer).

To prepare a print layer furnish, bleached hardwood kraft pulp (NBHK) and bleached softwood kraft pulp (NBSK) were mixed in a 70:30 dry weight ratio. Before the mixing, the NBHK and the NBSK were subjected to LC refining (50 and 120 kWh/tonne, respectively) such that both pulps obtained a °SR value of 25. Before the print layer headbox, rosin size (0.5 kg/tonne), alum (2 kg/tonne), strength agent (cationic starch, 5 kg/tonne), retention starch (3 kg/tonne), retention polymer (75 g/tonne), silica (300 g/tonne) and clay (55 kg/tonne) were added. In the print layer headbox, the consistency was 0.21% and the pH was 6.8.

To prepare a back layer furnish, unbleached softwood kraft pulp (UBK) and broke pulp were mixed in a 75:25 dry weight ratio. Before the mixing, the UBK and the broke pulp were subjected to LC refining to obtain °SR values of 23 and 30, respectively. Before the back layer headbox, AKD (0.5 kg/tonne), alum (0.4 kg/tonne), strength agent (cationic starch, 5 kg/tonne), retention starch (3 kg/tonne), retention polymer (75 g/tonne) and silica (300 g/tonne) were added. In the bottom layer headbox, the consistency was 0.18% and the pH was 7.5.

To prepare a middle layer furnish, broke pulp, NBSK and CTMP were mixed in a 45:10:45 dry weight ratio. Before the mixing, the pulps were subjected to LC refining to obtain the following values: °SR 30 for the broke pulp; °SR 20 for the NBSK and CSF 580 ml for the CTMP. Before the middle layer headbox, AKD (0.5 g/tonne), alum (0.3 g/tonne), strength agent (cationic starch, 4 kg/tonne), retention starch (3 kg/tonne), retention polymer (150 g/tonne) and silica (350 g/tonne) were added. In the middle layer headbox, the consistency was 0.32% and the pH was 7.5. The wire used for forming the middle layer included e.g. a top former and a breast roll shaker.

In the wire section, 0.7 g/m² starch was sprayed to each of the print layer web and the back layer web for ply-bond strength. At the end of the wire section, the three individual webs were couched together to form a three-layered web. In the press section arranged downstream the wire section, the three-layered web was pressed in three nips; a first double-felted shoe press nip followed by a second double-felted shoe press nip and a hard nip. The line load of the first double-felted shoe press nip was 656 kN/m. The line load of the second double-felted shoe press nip was 828 kN/m. The line load of the hard nip was 50 kN/m. The web speed in the press section was 854 m/min, which means that the press impulse of the whole press section was 108 kPa*s and that the total press impulse of the double-felted shoe press nips was 104 kPa*s.

Downstream the press section, the three-layered web was dried in a drying section (the steam consumption in this section was relatively low), subjected to calendering and then coated in a coating section according to the following: in a first blade coater, 8.5 g/m² of a pigment coating composition was applied to the surface of the print layer to form a first coating layer; and in a second blade coater, 11.5 g/m² of a pigment coating composition was applied to the first coating layer to form a second coating layer. Hence the total (dry) coat weight on the print layer surface was 20 g/m². Further, a very small amount (~0.3 g/m²) of starch was applied to the surface of the back layer in the coating section.

The properties of the resulting WTL product are presented in table 1 below. The properties are satisfactory.

**Table 1. "MD" means machine direction. "CD" means cross direction". "GM" means geometrical. "PS" means print side. "BS" means back side.**

| Property | Unit | Value |
|---|---|---|
| Grammage | g/m² | 202 |
| Caliper | µm | 252 |
| Density | kN/m | 800 |
| Tensile Strength MD | kN/m | 17.6 |
| Tensile Strength CD | kN/m | 12.6 |
| Stretch, MD | % | 2.0 |
| Stretch, CD | % | 6.2 |
| Bending Resistance Index GM | mNm⁶/g³ | 9.5 |
| SCT MD | kN/m | 6.1 |
| SCT CD | kN/m | 4.6 |
| Burst Strength | kPa | 734 |
| Scott Bond | J/m² | 336 |
| Z-strength | kPa | 593 |
| Brightness | D65 % | 79.9 |
| Roughness Bendtsen, PS | ml/min | 50 |
| Roughness, PS | PPS 1.0 | 1.5 |
| Cobb 60, PS | g/m² | 26 |
| Cobb 60, BS | g/m² | 33 |

Had the grammage been higher, the middle layer would have been a greater part of the whole board structure and the density would therefore have been lower. Further, the density would have been higher if the board was not pigment-coated.

### EXAMPLE 2

### Production of 270 g/m² LPB

Process data was collected from the production of three-layered liquid packaging board (LPB) over a period of about ten months. The production was carried out in the same paperboard machine as described in example 1 above, which means that a three-layered web was pressed in three nips: a first double-felted shoe press nip followed by a second double-felted shoe press nip and a hard nip. The production included coating (using two blade coaters) of the print layer with 7.5 + 11.5 g/m² of pigment coating composition. The back layer was coated with 0.4 g/m² of starch. Prior to coating, the three-layered web was subjected to calendering.

In the production, all layers were sized (internal sizing) with AKD, rosin size and alum. The amounts were about: 1 kg, 1.2 kg and 1.8 kg, respectively, for the print layer; 2.7 kg, 2.4 kg and 3.6 kg, respectively, for the middle layer; and 1 kg, 1 kg and 1.5 kg, respectively, for the back layer. Starch, retention polymer and silica were also added to the furnishes of the respective layers. For all layers, the headbox pH was about 7.0. The headbox consistency was about 0.25% for the print layer, about 0.55% for the middle layer and about 0.15% for the back layer. The grammage (gsm) was about 70 g/m² for the print layer and about 50 g/m² for the back layer. In the wire section, starch was sprayed to each of the print layer web and the back layer web for ply-bond strength.

Only data from production fulfilling the following criteria were considered:
- at least 70% unbleached kraft pulp in the back layer;
- at least 35% CTMP in the middle layer:
- more than 65% CTMP + broke pulp in the middle layer; and
- a machine speed in the press section of at least 650 m/min.

The data was clustered into two blocks of data: one block in which the total press impulse (PI) in the double-felted shoe press nips was at least 95 kPa*s and another block in which the press impulse in the double-felted shoe press nips was below 95 kPa*s (which is not part of the invention). Further details are provided in tables 2 and 3 below.

**Table 2. Average values from the "high PI" (≥ 95 kPa*s) block and the "low PI" (< 95 kPa*s) block. The low PI block is represented by the upper row and the high PI block is represented by the lower row. Both blocks had the same average bulk (1.42 cm³/g) and the same average bending resistance index (12.6 Nm⁶/kg³). "BHKP" means bleached hardwood kraft pulp. "BSKP" means bleached softwood kraft pulp. "BP" means broke pulp. "UB" means unbleached kraft pulp. "PL" means print layer. "ML" means middle layer. "BL" means back layer. "Bendt." means Bendtsen roughness (ml/min). The line load (kN/m) is given for the first and the second shoe press (SP1, SP2). MS means machine speed (m/min).**

| PI | gsm | PL | | ML | | | BL | PL | | BL | Line load | | MS |
|---|---|---|---|---|---|---|---|---|---|---|---|---|---|
| | | BHKP (%) | BSKP (%) | BSKP (%) | CTMP (%) | BP (%) | UB (%) | PPS (µm) | Bendt. | Bendt. | SP1 | SP2 | SP1 |
| 93 | 269.8 | 65.9 | 34.1 | 31.0 | 34.0 | 35.0 | 100 | 1.93 | 129 | 959 | 452 | 652 | 713 |
| 99 | 270.1 | 67.2 | 32.8 | 32.1 | 34.3 | 33.6 | 100 | 1.76 | 109 | 1004 | 454 | 649 | 670 |

The average °SR values of the pulps of the low PI block in table 2 are as follows: 25.6 for the PL BSKP; 28.9 for the PL BHKP; 26.4 for the ML BP; 17.4 for the ML BSKP; and 22.7 for the BL UB. The average CSF value of the ML CTMP of the low PI block was 612.5 ml. The average °SR values of the pulps of the high PI block in table 2 are as follows: 25.3 for the PL BSKP; 28.7 for the PL BHKP; 27.5 for the ML BP; 17.8 for the ML BSKP; and 22.0 for the BL UB. The average CSF value of the ML CTMP of the high PI block was 596.5 ml.

**Table 3. Median values from the "high PI" (≥ 95 kPa*s) block and the "low PI" (< 95 kPa*s) block. The low PI block is represented by the upper row and the high PI block is represented by the lower row. Both blocks had the same median bulk (1.42 cm³/g) and the same median bending resistance index (12.6 Nm⁶/kg³). The abbreviations are explained in table 1.**

| PI | gsm | PL | | ML | | | BL | PL | | BL | Line load | | MS |
|---|---|---|---|---|---|---|---|---|---|---|---|---|---|
| | | BHKP (%) | BSKP (%) | BSKP (%) | CTMP (%) | BP (%) | UB (%) | PPS (µm) | Bendt. | Bendt. | SP1 | SP2 | SP1 |
| 93 | 269.6 | 65.0 | 35.0 | 31.0 | 34.0 | 35.0 | 100 | 1.97 | 131 | 956 | 450 | 650 | 713 |
| 98 | 270.0 | 66.0 | 34.0 | 31.0 | 34.0 | 35.0 | 100 | 1.76 | 110 | 985 | 450 | 650 | 670 |

The median °SR values of the pulps of the low PI block in table 3 are as follows: 25.4 for the PL BSKP; 28.9 for the PL BHKP; 26.5 for the ML BP; 17.6 for the ML BSKP; and 22.7 for the BL UB. The median CSF value of the ML CTMP of the low PI block was 611.8 ml. The median °SR values of the pulps of the high PI block in table 3 are as follows: 25.2 for the PL BSKP; 28.6 for the PL BHKP; 27.5 for the ML BP; 17.9 for the ML BSKP; and 22.0 for the BL UB. The median CSF value of the ML CTMP of the high PI block was 592.1 ml.

A higher press impulse did not reduce the bulk according to tables 2 and 3.

As shown in table 3, the median Bendtsen roughness of the print layer was 131 ml/min when the median press impulse over the shoe presses was 93 kPa*s and 110 ml/min when the median press impulse over the shoe presses was 98 kPa*s. If average values are instead considered, about the same results are obtained (see table 2). Further, an increased press impulse reduces the print layer PPS according to tables 2 and 3. The press impulse increase is thus connected to improved surface properties of the print layer.

Interestingly, a correlation between increased press impulse and decreased Bendtsen roughness is not seen for the back layer. Instead, the back layer actually has a slightly higher Bendtsen roughness when the press impulse is higher. This suggests that the mechanism behind the print layer improvements is related to coatability. Without being bound by any specific scientific theory, the inventor believes that a higher press impulse in the double-felted shoe presses results in a denser surface that absorbs less of the coating composition applied in the coating section and that less absorption results in better coverage and hence a finer surface. The increased press impulse may thus have an effect similar to that of a size press, which is often arranged upstream the coating section in a paperboard machine.

## Claims

1. A method of producing a paper- or linerboard having a grammage measured according to ISO 536:2019 of 170-310 g/m² and comprising a print layer, a middle layer and a back layer, wherein the middle layer is formed from a middle layer furnish comprising at least 30% by dry weight CTMP and at least 20% by dry weight broke pulp and the back layer is formed from a back layer furnish comprising at least 60% by dry weight of an unbleached kraft pulp, said method comprising the step of subjecting a multi-layered web at a speed of at least 600 m/min to pressing in a press section comprising a first and a second double-felted shoe press nip arranged in series, wherein the total press impulse of the double-felted shoe press nips is at least 95 kPa*s, preferably at least 100 kPa*s,
and wherein CTMP and broke pulp together constitute at least 65% by dry weight of the middle layer furnish
and wherein the press section comprises a further nip arranged downstream the double-felted shoe press nips, which further nip is a hard nip or a single-felted shoe press nip, in which single-felted shoe press nip the felt is contacting the back side and wherein the print layer is coated with a composition comprising at least one pigment and at least one binder, which coating step comprises a plurality of substeps, each applying a sublayer and wherein the total amount (dry weight) of coating applied in the coating step is 11-30 g/m²
and wherein the paper- or linerboard is subjected to hard nip calendering prior to the coating step but after a drying section
and wherein the method comprises no calendering step after the coating step
and wherein the pigment-coated the print side of the paper- or linerboard has a PPS 1.0 roughness measured according to ISO 8791-4:2013 (soft backing & 1000 kPa clamping pressure) of below 1.8 µm.

2. The method of claim 1, wherein the speed is at least 650 m/min, such as at least 700 m/min, such as at least 750 m/min.

3. The method of claim 1 or 2, wherein the line load of the second double-felted shoe press nip is higher than the line load of the first double-felted shoe press nip.

4. The method of any one of the preceding claims, wherein the head box consistency of the middle layer furnish is 0.15% - 0.42%, such as 0.25% - 0.40%.

5. The method of any one of the preceding claims, wherein the head box consistency of the print layer furnish is 0.12% - 0.25%.

6. The method of any one of the preceding claims, wherein the head box consistency of the back layer furnish is 0.12% - 0.25%.

7. The method of any one of the preceding claims, wherein the middle layer furnish comprises at least 35% by dry weight CTMP, such as at least 40% by dry weight CTMP.

8. The method of any one of the preceding claims, wherein the middle layer furnish further comprises at least 30% by dry weight broke pulp.

9. The method of claim 8, wherein CTMP and broke pulp together constitute at least 75% by dry weight of the middle layer furnish.

10. The method of any one of the preceding claims, wherein the middle layer furnish further comprises kraft pulp.

11. The method of any one of the preceding claims, wherein the print layer furnish comprises a mixture of hardwood kraft pulp and softwood kraft pulp.

12. The method of claim 11, wherein hardwood kraft pulp and softwood kraft pulp together constitute at least 80% by dry weight of the print layer furnish, such as at least 90% by dry weight of the print layer furnish.

13. The method of any one of the preceding claims, wherein the back layer furnish further comprises broke pulp.

14. The method of claim 13, wherein unbleached kraft pulp and broke pulp together constitute at least 80% by dry weight of the back layer furnish, such as at least 90% by dry weight of the back layer furnish.

15. The method of any one of the preceding claims, wherein the forming of the middle layer comprises use of a breast roll shaker.

## Patentansprüche

1. Verfahren zur Herstellung von Papier- oder Deckenpapier mit einem nach ISO 536:2019 gemessenen Flächengewicht von 170-310 g/m² und aufweisend eine Druckschicht, eine Mittelschicht und eine Rückschicht, wobei die Mittelschicht aus einem Mittelschichtstoff gebildet ist, der mindestens 30 Gew.-% CTMP und mindestens 20 Gew.-% Rücklaufzellstoff auf Trockengewichtsbasis aufweist, und wobei die Rückschicht aus einem Rückschichtstoff gebildet ist, der mindestens 60 Gew.-% eines ungebleichten Kraftzellstoffs auf Trockengewichtsbasis aufweist, das Verfahren aufweisend den Schritt des Unterziehens eines mehrlagigen Bahnmaterials einem Pressen mit einer Geschwindigkeit von mindestens 600 m/min in einem Pressenabschnitt, der einen ersten und einen zweiten doppelt befilzten Schuhpressspalt aufweist, die in Serie angeordnet sind, wobei der gesamte Pressimpuls der doppelt befilzten Schuhpressspalte mindestens 95 kPa·s, bevorzugt mindestens 100 kPa·s beträgt,
und wobei CTMP und Rücklaufzellstoff zusammen mindestens 65 Gew.-% des Mittelschichtstoffs auf Trockengewichtsbasis bilden,
und wobei der Pressenabschnitt einen zusätzlichen, stromabwärts der doppelt befilzten Schuhpressspalte angeordneten Pressspalt aufweist, welcher zusätzliche Pressspalt ein harter Pressspalt oder ein einfach befilzter Schuhpressspalt ist, bei welchem einfach befilzten Schuhpressspalt das Filzmaterial mit der Rückseite in Kontakt steht, und wobei die Druckschicht mit einer Zusammensetzung beschichtet ist, die mindestens ein Pigment und mindestens ein Bindemittel aufweist, wobei der Beschichtungsschritt eine Mehrzahl von Teilschritten aufweist, in jedem von denen eine Teilschicht aufgebracht wird, und wobei die Gesamtmenge (Trockengewicht) der im Beschichtungsschritt aufgebrachten Beschichtung 11-30 g/m² beträgt,
und wobei das Papier- oder Deckenpapier vor dem Beschichtungsschritt, jedoch nach einem Trocknungsabschnitt, einer Hartkalanderung unterzogen wird,
und wobei das Verfahren keinen Kalanderungsschritt nach dem Beschichtungsschritt aufweist,
und wobei die pigmentbeschichtete Druckseite des Papier- oder Deckenpapiers eine PPS-1,0-Rauigkeit, gemessen gemäß ISO 8791-4:2013 (weiche Unterlage und 1000 kPa Anpressdruck), von weniger als 1,8 µm aufweist.

2. Verfahren nach Anspruch 1, wobei die Geschwindigkeit mindestens 650 m/min beträgt, beispielsweise mindestens 700 m/min, beispielsweise mindestens 750 m/min.

3. Verfahren nach Anspruch 1 oder 2, wobei die Linienlast des zweiten doppelt befilzten Schuhpressspalts größer ist als die Linienlast des ersten doppelt befilzten Schuhpressspalts.

4. Verfahren nach einem der vorhergehenden Ansprüche, wobei die Konsistenz des Mittelschichtstoffs im Stoffauflauf 0,15 % bis 0,42 % beträgt, beispielsweise 0,25 % bis 0,40 %.

5. Verfahren nach einem der vorhergehenden Ansprüche, wobei die Konsistenz des Druckschichtstoffs im Stoffauflauf 0,12 % bis 0,25 % beträgt.

6. Verfahren nach einem der vorhergehenden Ansprüche, wobei die Konsistenz des Rückschichtstoffs im Stoffauflauf 0,12 % bis 0,25 % beträgt.

7. Verfahren nach einem der vorhergehenden Ansprüche, wobei der Mittelschichtstoff mindestens 35 Gew.-% CTMP aufweist, beispielsweise mindestens 40 Gew.-% CTMP, auf das Trockengewichtsbasis.

8. Verfahren nach einem der vorhergehenden Ansprüche, wobei der Mittelschichtstoff ferner mindestens 30 Gew.-% Rücklaufzellstoff auf Trockengewichtsbasis aufweist.

9. Verfahren nach Anspruch 8, wobei CTMP und Rücklaufzellstoff zusammen mindestens 75 Gew.-% des Mittelschichtstoffs auf Trockengewichtsbasis bilden.

10. Verfahren nach einem der vorhergehenden Ansprüche, wobei der Mittelschichtstoff ferner Kraftzellstoff aufweist.

11. Verfahren nach einem der vorhergehenden Ansprüche, wobei der Druckschichtstoff eine Mischung aus Hartholz-Kraftzellstoff und Weichholz-Kraftzellstoff aufweist.

12. Verfahren nach Anspruch 11, wobei Hartholz-Kraftzellstoff und Weichholz-Kraftzellstoff zusammen mindestens 80 Gew.-% des Druckschichtstoffs auf Trockengewichtsbasis bilden, beispielsweise mindestens 90 Gew.-% des Druckschichtstoffs auf Trockengewichtsbasis.

13. Verfahren nach einem der vorhergehenden Ansprüche, wobei der Rückschichtstoff ferner Rücklaufzellstoff aufweist.

14. Verfahren nach Anspruch 13, wobei ungebleichter Kraftzellstoff und Rücklaufzellstoff zusammen mindestens 80 Gew.-% des Rückschichtstoffs auf Trockengewichtsbasis bilden, beispielsweise mindestens 90 Gew.-% des Rückschichtstoffs auf Trockengewichtsbasis.

15. Verfahren nach einem der vorhergehenden Ansprüche, wobei die Bildung der Mittelschicht die Verwendung eines Brustwalzenschüttlers aufweist.

## Revendications

1. Procédé de fabrication d'un papier ou d'un carton doublure ayant un grammage mesuré selon la norme ISO 536:2019 compris entre 170 et 310 g/m² et comprenant une couche imprimée, une couche intermédiaire et une couche arrière, dans lequel la couche intermédiaire est formée à partir d'une pâte pour couche intermédiaire comprenant au moins 30 % en poids sec de pâte CTMP et au moins 20 % en poids sec de pâte de broyage, et la couche arrière est formée à partir d'une pâte pour couche arrière comprenant au moins 60 % en poids sec de pâte kraft non blanchie, ledit procédé comprenant l'étape consistant à soumettre une bande multicouche à une vitesse d'au moins 600 m/min à un pressage dans une section de presse comprenant une première et une deuxième presses à double feutre pour sabot disposées en série, dans lequel l'impulsion de pressage totale des presses à double feutre pour sabot est d'au moins 95 kPa*s, de préférence d'au moins 100 kPa*s,
et dans lequel la pâte CTMP et la pâte de broyage constituent ensemble au moins 65 % en poids sec de la charge de la couche intermédiaire,
et dans lequel la section de presse comprend une autre ligne de contact disposée en aval des presses à double feutre pour sabot, cette autre ligne de contact est une ligne de contact dure ou une presse à simple feutre pour sabot,
dans laquelle presse à simple feutre pour sabot, le feutre est mis en contact avec la face arrière et dans lequel la couche d'impression est revêtue d'une composition comprenant au moins un pigment et au moins un liant, cette étape de revêtement comprenant une pluralité de sous-étapes, chacune appliquant une sous-couche et dans lequel la quantité totale (en poids sec) de revêtement appliquée dans l'étape de revêtement est comprise entre 11 et 30 g/m²
et dans lequel le papier ou le carton doublure est soumis à un calandrage à pincement dur avant l'étape de revêtement mais après une section de séchage
et dans lequel le procédé ne comprend aucune étape de calandrage après l'étape de revêtement
et dans lequel le côté imprimé revêtu de pigment du papier ou du carton doublure a une rugosité PPS 1,0 mesurée selon la norme ISO 8791-4:2013 (support souple et pression de serrage de 1 000 kPa) inférieure à 1,8 µm.

2. Procédé selon la revendication 1, dans lequel la vitesse est d'au moins 650 m/min, telle qu'au moins 700 m/min, telle qu'au moins 750 m/min.

3. Procédé selon la revendication 1 ou la revendication 2, dans lequel la charge linéaire de la deuxième presse à double feutre pour sabot est supérieure à la charge linéaire de la première presse à double feutre pour sabot.

4. Procédé selon l'une quelconque des revendications précédentes, dans lequel la consistance de la pâte à papier de la couche intermédiaire dans la caisse de tête est comprise entre 0,15 % et 0,42 %, telle que comprise entre 0,25 % et 0,40 %.

5. Procédé selon l'une quelconque des revendications précédentes, dans lequel la consistance de la pâte à papier de la couche d'impression dans la caisse de tête est comprise entre 0,12 % et 0,25 %.

6. Procédé selon l'une quelconque des revendications précédentes, dans lequel la consistance de la pâte à papier de la couche arrière dans la caisse de tête est comprise entre 0,12 % et 0,25 %.

7. Procédé selon l'une quelconque des revendications précédentes, dans lequel la pâte de la couche intermédiaire comprend au moins 35 % en poids sec de pâte CTMP, tel qu'au moins 40 % en poids sec de pâte CTMP.

8. Procédé selon l'une quelconque des revendications précédentes, dans lequel la pâte de la couche intermédiaire comprend en outre au moins 30 % en poids sec de pâte de broyage.

9. Procédé selon la revendication 8, dans lequel la pâte CTMP et la pâte de broyage constituent ensemble au moins 75 % en poids sec de la pâte de la couche intermédiaire.

10. Procédé selon l'une quelconque des revendications précédentes, dans lequel la pâte de la couche intermédiaire comprend en outre de la pâte kraft.

11. Procédé selon l'une quelconque des revendications précédentes, dans lequel la pâte de la couche d'impression comprend un mélange de pâte kraft de bois dur et de pâte kraft de bois tendre.

12. Procédé selon la revendication 11, dans lequel la pâte kraft de bois dur et la pâte kraft de bois tendre constituent ensemble au moins 80 % en poids sec de la composition de la couche d'impression, tel qu'au moins 90 % en poids sec de la composition de la couche d'impression.

13. Procédé selon l'une quelconque des revendications précédentes, dans lequel la composition de la couche arrière comprend en outre de la pâte de broyage.

14. Procédé selon la revendication 13, dans lequel la pâte kraft non blanchie et la pâte de broyage constituent ensemble au moins 80 % en poids sec de la pâte de la couche arrière, tel qu'au moins 90 % en poids sec de la pâte de la couche arrière.

15. Procédé selon l'une quelconque des revendications précédentes, dans lequel la formation de la couche intermédiaire comprend l'utilisation d'un agitateur à rouleaux.
